

Oct. 15, 1957

J. U. KOREE

2,809,904

SMOKING PRODUCT

Filed Nov. 17, 1954



INVENTOR.  
JEAN U. KOREE  
BY  
*Albert Sperry*  
ATTORNEY

1

2,809,904

## SMOKING PRODUCT

Jean U. Koree, New York, N. Y., assignor to The Raymar Company, New York, N. Y., a corporation of New York

Application November 17, 1954, Serial No. 469,371

5 Claims. (Cl. 131—2)

This invention relates to a new type of smoking product and is directed particularly to products consisting essentially of bagasse and to methods of producing and using such products.

In my issued Patent No. 2,576,021, I have described a tobacco substitute consisting of paper made from long and short fibers of bagasse and containing agents which impart to the smoke from such paper, a flavor and aroma similar to that of natural tobacco.

I have now discovered that when bagasse is ground in a ball mill or the like until it is largely reduced to a colloidal condition of the corpuscular type, and is thereafter formed into an integral sheet, the smoke produced on burning thereof possesses a new and characteristic tang and flavor and a pleasing new aroma. The smoke differs materially from that of tobacco or from any other product with which I am acquainted. It has somewhat the flavor of tea or sage and is smooth, brisk or tangy and very pleasing and satisfying in effect. Moreover, the smoke differs materially from that produced when the bagasse is in a fibrous condition when burned. It is quite possible that the difference in the amount, character, flavor and aroma of the smoke is due to the fact that bagasse fibers present a very extensive surface area as compared with their volume and, accordingly, when burned, they undergo a different and more rapid type of combustion. The smoke resulting from fibrous bagasse is of a different and more acrid type and contains acroleins and irritation producing aldehydes. Moreover, the rapid burning of bagasse fibers apparently destroys or impairs certain of the aromatic or flavor imparting ingredients contained in bagasse. In contrast, the smoke produced on burning of a non-fibrous sheet wherein most or all of the bagasse is in a corpuscular colloidal condition is smooth and tangy but non-irritating. It is not a tobacco-like smoke but, instead, possesses its own characteristic flavor and aroma which is pleasant and enjoyable. Moreover, tobacco smoke has a pH value above 7 and generally about 8 or 9 whereas I find that the smoke from colloidal bagasse films has a pH below 7 and generally about 4 or 5. Furthermore, the smoke does not contain nicotine or the tars and constituents of tobacco smoke which are generally believed to be injurious to health.

It is an object of the present invention to produce a new type of smoking product which consists essentially of non-fibrous integral sheets or shreds of bagasse.

Another object of the invention is to provide novel methods for producing integral sheets or shreds of bagasse wherein the bagasse is largely in the form of corpuscular colloidal particles.

A further object of the invention is to produce a smoking product consisting essentially of bagasse and having the property when burned of producing a smoke having a characteristic flavor and aroma differing materially from that of tobacco or fibrous bagasse.

These and other objects and features of the present invention will appear from the following description thereof wherein reference is made to the flow diagram of the accompanying drawing.

The bagasse product of the present invention is preferably produced by grinding the bagasse with water or other liquid in a ball mill or colloid mill or by otherwise

2

treating the bagasse so as to reduce it to a colloidal condition of the corpuscular type. The resulting slurry containing colloidal bagasse is thereafter cast or otherwise formed into a film and the water or liquid is removed whereby a continuous integral sheet of bagasse is produced. The product contains substantially all of the original constituents of the bagasse in a chemically unaltered state or in such a condition that the full flavor and aroma of the product is preserved.

10 The resulting sheet of corpuscular colloidal bagasse may be shredded or otherwise comminuted to form a product suitable for smoking in a pipe or adapted to be formed into cigarettes with a wrapper of cigarette paper or a wrapper formed of the bagasse sheet material itself. The 15 sheeted material also may be used as a wrapper for tobacco similar to the conventional cigarette paper or the sheet may be wrapped and folded to form cigars or similar products which, when smoked, will possess the characteristic aroma and flavor of bagasse as distinguished 20 from tobacco. The sheets further may be compacted into a mass for use as a chewing product or it may be comminuted and ground into a powder usable in the same manner as snuff.

In forming the sheet material of the present invention, 25 the bagasse is preferably ground up or chopped into short lengths by attrition or otherwise and thereafter is ground in a ball mill with water for from 2 to 16 hours. If the bagasse is ground for less than about 2 hours, the sheet material thereafter formed contains an excessive amount 30 of undestroyed fibers which impair the properties of the sheet itself and further impair the flavor and aroma of the smoke produced on burning the material. On the other hand, if the bagasse is ground in a ball mill for more than about 16 hours, the product is not materially 35 improved whereas the cost of manufacture is considerably increased.

The amount of water used in carrying out the colloiding operation does not appear to be very important provided it is sufficient to produce a slurry of suitable consistency.

40 Generally, at least 5 and preferably about 8 parts by weight of water are used for each part of bagasse. Moreover, agents which accelerate hydration or gelling of the cellulose may be added to the water. For this purpose, I may use ammonia, calcium hydroxide, or mild acids 45 such as acetic, lactic or tartaric acid. Further, it is sometimes desirable to add a combustible film forming agent to increase the strength and flexibility of the sheet produced. Typical agents of this character are polyvinyl alcohol, gelatin, carboxy methyl cellulose, carboxy ethyl cellulose, 50 starch, vegetable glues, agar, elemi, gum tragacanth, and the like. These substances may be added in amounts varying from 1 to 20% by weight based upon the weight of the dry bagasse in the product. Agents also may be added to the film forming slurry to alter the burning characteristics of the product. Thus, for example, sodium or potassium nitrate or hydrated alumina, ammonium borate or other combustion controlling agents may be added to the composition in suitable amounts up to 10% by weight 55 of the bagasse for varying the rate of combustion of the product.

It is also desirable, in some instances, to add hygroscopic materials or humectants to the product to prevent drying out of the sheet when formed. For this purpose, glycerine, diethylene glycol and the like may be added to 60 the material during the grinding or disintegration thereof, or they may be added to the resulting slurry before the material is formed into a film and dried to form a sheet. Such agents also may be sprayed on to the finished sheet if desired, and such spraying of the sheet material is some- 65 times preferred since hygroscopic materials tend to retard the drying and sheet formation of the films from which the product is produced.

For some purposes, and particularly when a relatively heavy ash is desired, the composition may include inert filler materials such as finely divided clay, bentonite, kieselguhr, calcium carbonate, zinc oxide or the like. Such fillers may be added in amounts up to 5% by weight based upon the weight of the bagasse. They are preferably added while the bagasse is undergoing treatment in the ball mill in order that they may be uniformly distributed and incorporated in the colloidal composition.

In producing a slurry for casting into a film the product from the ball mill or colloid mill may, if desired, be filtered after incomplete or limited grinding or dispersion of the bagasse and the coarse or partially ground material remaining on a 60 mesh screen, for example, may be returned to the ball mill while the liquid containing the colloidal or dispersed bagasse may be used in forming a film. However, when bagasse is ground in a ball mill for 4 to 6 hours or more, such filtering is not generally necessary since the major portion of the bagasse is usually dispersed.

In order to illustrate typical procedure in accordance with the present invention, the process may be carried out as indicated by the flow sheet of the drawing. If desired, the bagasse may first be washed to eliminate water soluble constituents although washing is not necessary and the loss of sugars may even be detrimental. It is then ground or comminuted so as to shorten the period required to reduce the bagasse to a colloidal condition. The bagasse is thereafter subjected to treatment in a ball mill with about 8 times its weight of water. Grinding in the ball mill serves to break up the fibers into short lengths such that the bagasse is largely reduced to the form of corpuscular colloidal particles. This may be effected provided the grinding is continued for from 2 to 16 hours and preferably about 4 hours. The temperature at which the colloidizing operation is carried out is preferably in the range from about 20° C. to 70° C. and conveniently can be conducted at room temperature.

The resulting slurry is thereafter cast or spread in a film upon a conveyor, rotating drum or other film forming device, and the water is evaporated by mild heating with or without the use of reduced pressure. The film thereby obtained may then be cut or shredded to form the desired pieces for use in producing the smoking product.

In a typical composition produced as indicated in the flow sheet of Fig. 1, a ball mill is charged with 125 parts of ground bagasse and 1000 parts by weight of water to which are added 20 parts by weight of water soluble polyvinyl alcohol and 40 parts by weight of glycerine. After 4 hours of grinding in the ball mill, this composition was sheeted whereby a continuous sheet was obtained wherein substantially all of the bagasse was in a colloidal condition of the corpuscular type. The sheet had excellent flexibility and was sufficiently strong to permit it to be shredded into a form suitable for smoking. The shredded material was enclosed within a wrapper forming a cigarette-like product which, when smoked, had a very pleasant, brisk or tangy and characteristic aroma and flavor differing fundamentally from that of tobacco. Moreover, the smoke contains no nicotine and but little tars or stain producing constituents. Moreover, no harmful, toxic or other constituents injurious to health have been found in the smoke.

The methods by which the products of the present invention may be produced are, in general, the same or similar to those employed in producing certain tobacco products since the bagasse may be ground in a ball mill such as that used in the methods described in the patents to Wells et al. No. 2,433,877 and Sowa et al. No. 2,485,670, issued January 6, 1948 and October 25, 1949, respectively. However, the material employed in producing colloidal films having the characteristic and desirable smoking and physical properties of the present invention is bagasse. Nevertheless, the grinding steps and methods of procedure described in said patents may be used to advantage in

treating bagasse to produce an entirely new and different type of smoking product which is devoid of tobacco, nicotine and most, if not all, of the constituents of tobacco which are said to be injurious to health.

5 The product of the present invention is therefore desirable as a pleasant and relaxing smoking material which may be employed in the form of cigarettes, cigars or a pipe smoking material. It may further be used as a chewing product or as a powdered product usable in the same manner as snuff.

The particular form and size of the sheets or shreds of material and the thickness thereof can, of course, be varied. Furthermore, the amount of colloidal material contained in the product may be varied by increasing or 15 decreasing the period of grinding or treatment in a ball mill, colloid mill or other dispersing equipment used. In general, it is desirable to have at least 50% of the bagasse in a colloidal form of the corpuscular type in the film. For best results, 70% or more of the product should be 20 in the corpuscular colloidal type and the balance should consist of fibers of minute dimensions.

While the compositions of the present invention preferably consist substantially entirely of bagasse it will be apparent that a minor percentage of film forming material, 25 humectants, fillers and the like may be present. Conventional flavoring agents, sweetening agents and "casing" agents also may be used for the purpose of imparting desired physical properties to the product, whereas special agents for altering or improving the flavor, aroma or other 30 characteristics to the smoke may be added to the product. Nevertheless, for most purposes, the only vegetable material contained in the product is bagasse and it is the colloidal bagasse of the corpuscular type which constitutes the principal smoke forming and aroma and taste imparting 35 properties to the product.

It will thus be apparent that the methods of production and the composition of the product are capable of considerable variation without departing from the spirit and scope of the invention.

40 What I claim is:

1. A tobacco substitute, the major portion of which consists of bagasse in corpuscular colloidal form.

2. A tobacco substitute wherein the sole vegetable material consists of bagasse, at least 50% of which is in 45 a corpuscular colloidal dispersed form.

3. The method of producing a tobacco substitute which comprises the steps of subjecting bagasse to a dispersing operation by grinding in an aqueous medium until at least 50% of the bagasse is reduced to a corpuscular colloidal condition, casting the resulting dispersion into the form of a film, and drying said film.

4. A tobacco substitute consisting of sheeted colloidal dispersed bagasse wherein the major portion of the bagasse is in the form of corpuscular type colloidal particles.

5. A tobacco substitute comprising bagasse which has been ground in an aqueous medium until reduced to a corpuscular type of colloid, and thereafter sheeted and dried.

#### References Cited in the file of this patent

#### UNITED STATES PATENTS

|           |                    |               |
|-----------|--------------------|---------------|
| 1,894,577 | Wells              | Jan. 17, 1933 |
| 2,576,021 | Korec              | Nov. 20, 1951 |
| 2,592,553 | Frankenburg et al. | Apr. 15, 1952 |

#### OTHER REFERENCES

Hauser: "Colloid Phenomena," published 1939 by McGraw-Hill Book Co., New York. Pages 34, 35 and 36.

Hauser: "Colloidal Phenomena," published 1939 by McGraw-Hill Book Co., Inc., New York. Pages 25 and 194.

Hartman: "Colloid Chemistry," published 1947 by Houghton Mifflin Co., New York. Second edition, page 453.